

# UNITED STATES PATENT OFFICE.

EMILE BRONNERT, OF NIEDERMORSCHWEILER, NEAR MULHAUSEN, GERMANY,  
ASSIGNOR, BY MESNE ASSIGNMENTS, TO THE CHEMICAL FOUNDATION, INC.,  
A CORPORATION OF DELAWARE.

## PROCESS FOR THE MANUFACTURE OF LUSTROUS THREADS FROM CRUDE VISCOSE BY MEANS OF WARM MINERAL ACIDS.

1,414,070.

Specification of Letters Patent. Patented Apr. 25, 1922.

No Drawing.

Application filed January 8, 1914. Serial No. 811,060.

*To all whom it may concern:*

Be it known that I, EMILE BRONNERT, a subject of the Emperor of Germany, residing at Niedermorschweiler, near Mulhausen, Alsace, Germany, have invented certain new and useful Improvements in Processes for the Manufacture of Lustrous Threads from Crude Viscose by Means of Warm Mineral Acids; and I do hereby declare the following to be a full, clear, and exact description of the invention.

This invention relates to processes for the manufacture of lustrous threads (artificial silk), sheets, films, and the like from crude viscose, by the use of warm mineral acids, and aims to provide improvements in such processes, and in the articles produced thereby.

British Patent 17503/1902 recommends the use of a 10 per cent solution of sulphuric acid for the spinning of crude viscose (Rohviscose), stating that the sulphur separating out on the decomposition of the viscose can be subsequently again removed with sodium sulphide. The process, however, found no application, since the de-sulphured threads were brittle and had but little luster.

The same inventor states also in German Patent 200023/1907, that it is not possible to use crude viscose for spinning in sulphuric acid and recommends a separate previous precipitation and purifying of the crude viscose.

Other authors also had already (British Patent 2529/1902) recognized the like impossibility of the application of sulphuric acid as a precipitating medium for crude viscose and had recommended special preliminary precipitations and purification of the same in order to be able to use dilute sulphuric acid or salts furnishing sulphuric acid, and preferably at twenty degrees centigrade, as a precipitating bath. German Patent 187947/1905 had for the first time found another way in which to employ the sulphuric acid for the spinning of crude viscose. This means consisted in adding a predetermined amount of the salt of the acid, to thus remove the violence of the decomposition reaction and to allow the thread to be produced under more favorable conditions. Later it was found that glucose and other organic bodies acted similarly to salts upon

the acid and consequently upon the threads produced.

In a surprising manner it has now been shown that the crude viscose can be also spun with a mineral acid, such as sulphuric acid, without any addition, if on the one hand concentration and temperature of the acid are adapted to the age of the viscose to be employed.

In general, the crude viscose must be so much the older as the acid chosen is more concentrated and warmer.

The methods of determination of the necessary condition of the viscose solution in each single case are unfortunately too unreliable to be recommended. If, however, the alkali cellulose has been left to itself in the well-known manner first for two or three days at about 20° to 25° C. and then the viscose solution made therefrom has been left for a certain number of days at a constant temperature of from 17° to 22° centigrade, then the same conditions can at any time be easily again produced which are necessary for assuring a constantly equal product, and which have been recognized once for all as such by means of expert methodical preliminary experiments.

*Example I.*—Crude viscose which has stood about eight days or more at 15° to 20° centigrade and has been several times filtered is forced into warm sulphuric acid of a strength of 20 per cent at 40° C., wound on suitable bobbins, and then or afterwards washed with warm water and in well known manner under tension dried and de-sulphured.

*Example II.*—Crude viscose which has stood about four days or longer at 15° to 20° C. after filtering is forced into 10 per cent acid at a temperature of 25° C. or warmer or of equivalent quantity of another mineral acid while drawing the thread through it for a length, for example, of only three centimeters, and then, as in Example I, again washed and dried and de-sulphured under tension.

I claim as my invention:

1. Process for the manufacture of lustrous threads from viscose comprising directly transforming crude viscose into such threads by forcing it in the form of a correspondingly shaped stream into a thread

forming coagulating bath consisting of a dilute mineral acid of somewhat high temperature, about 25° to 50° C., the crude viscose employed being so much the older as the acid employed is stronger and warmer, the thus formed thread being capable of being wound upon suitable bobbins.

2. A process for the production of lustrous threads from viscose comprising allowing crude viscose to stand about eight days or more under 15 to 20 degrees C. temperature, filtering, and forcing it into a

warm bath of sulphuric acid of about 20% concentration and about 40 degrees C. temperature, winding upon suitable bobbins, 15 washing with warm water in well known manner, drying and desulphuring.

In witness whereof, I have hereunto signed my name in the presence of two subscribing witnesses.

EMILE BRONNERT.

Witnesses:

PHILIP HOLLAND,  
ARNOLD ZUBER.